

1

3,184,410

**MOLYBDENUM COMPOUNDS AND LUBRICATING COMPOSITIONS CONTAINING THEM**

Leslie Bretherick, Windsor, England, assignor to The British Petroleum Company Limited, London, England, a corporation of England

No Drawing. Filed Aug. 5, 1964, Ser. No. 387,786

Claims priority, application Great Britain, Aug. 20, 1963, 32,871/63

7 Claims. (Cl. 252—42.7)

This invention relates to novel molybdenum compounds having utility as lubricants and as additives therefore, and to lubricating compositions containing such compounds.

Although molybdenum disulphide ( $\text{MoS}_2$ ) behaves as a good solid lubricant (i.e., in the absence of liquid lubricant), lubricating oils containing finely divide molybdenum disulphide in suspension show little advantage under normal conditions over the base oils. This may be due to the fact that molybdenum disulphide is insoluble in mineral oils or esters.

Oil-soluble compounds containing both molybdenum and sulphur have been proposed as additives to improve the load carrying properties of lubricants. Examples of such oil-soluble compounds are certain molybdenum alkyl xanthates and molybdenum dialkyldithiophosphates. Such compounds appear to decompose at the high temperatures and pressures encountered under frictional stress with the deposition of compounds containing molybdenum, sulphur and, usually, oxygen, e.g.,  $\text{MoOS}_2$  and  $\text{MoO}_2\text{S}$ . The solid lubricating properties of these latter compounds are not as good as those of molybdenum disulphide.

I have now discovered certain novel molybdenum compounds which are soluble in mineral and synthetic lubricating oils and which improve the load carrying or anti-wear properties of such oils.

The invention therefore, according to one aspect, consists in novel compounds of the general formula



where  $\text{R}_1$  and  $\text{R}_2$ , which may be the same or different, are alkyl, alkenyl, or alkynyl groups preferably having 1-20 carbon atoms, and the  $\text{X}$ 's are oxygen or sulphur atoms, at least one of the  $\text{X}$ 's being an oxygen atoms. Where  $\text{R}_1$  and/or  $\text{R}_2$  are alkenyl or alkynyl groups, the group(s) may contain more than one multiple bond. Preferably however,  $\text{R}_1$  and  $\text{R}_2$  are alkyl groups, especially branched chain alkyl groups. It is to be understood of course that the invention includes products consisting of a mixture of different compounds in accordance with Formula I.

The invention also includes a method of preparing compounds of Formula I in which a compounds of the formula



2

where the  $\text{X}$ 's are oxygen or sulphur atoms, at least one of the  $\text{X}$ 's in each ring being an oxygen atom, and  $\text{R}_1$  and  $\text{R}_2$  have the values stated previously, is reacted with sulphur, in an inert atmosphere and preferably in a solvent, e.g., the diketone shown chelated in Formula I, and at elevated temperature, e.g., 100°-200° C. Compounds of Formula II are known and commercially available. The diketone produced as a by-product of the reaction may be recovered for re-use, e.g., by distillation.

- 10 The invention further includes a method of preparing compounds of Formula I in which molybdenum hexacarbonyl is reacted with sulphur and a diketone or mono-thio diketone of the Formula  $\text{R}_1\text{C}(\text{XCH}_2\text{C}(\text{X})\text{R}_2$  where  $\text{X}$ ,  $\text{R}_1$  and  $\text{R}_2$  have the values stated previously for Formula I. This method of preparation has the advantage over the previous method that it avoids using the air-sensitive compounds of Formula II and the reaction mixture generates its own inert atmosphere of carbon monoxide.
- 15 20 According to a further aspect of the invention there is provided a lubricating composition consisting essentially of a blend of a lubricating oil, which may be mineral or synthetic, and a molybdenum compound of Formula I. For most applications, e.g., for use as an engine or gear lubricant, only a small proportion, e.g., 0.1-5% by weight of the composition, of the molybdenum compound will be needed in the blend to confer improved load carrying or anti-wear properties on the lubricating oil. The amount of molybdenum compound that can be dissolved in the lubricating oil will depend primarily on the nature of the alkyl groups  $\text{R}$  and it is to be understood that the composition may contain suspended as well as dissolved molybdenum compound of Formula I. In the use of such a lubricating composition, the dissolved molybdenum compound will gradually be converted to molybdenum disulphide and other compounds and at the same time a corresponding amount of the undissolved material will go into solution.
- 25 30 35 40 45 50 55

Actual preparations of a number of compounds in accordance with the invention will now be described by way of example only.

### EXAMPLE 1

Sample quantities of dithiomolybdenyl acetylacetone were prepared by each of the two general methods of the invention. Actual preparative details are given as Method 1 and Method 2 below.

#### Method 1

50 A mixture of molybdenum tri-acetylacetone (3.93 g.) prepared by the method of Larson and Moore (J. Inorg. Chem. 1, 856, 1952), acetylacetone (25 ml.) and sublimed sulphur (0.64 g.) was stirred and refluxed in an inert atmosphere for 5 hours. The black mixture was freed of solvent by vacuum distillation and the residue dispersed in benzene. The black solid was filtered off, washed with benzene and dried in vacuo.

The yield was 1.7 gm.  
The product so recovered is hereinafter referred to as M1.

The reaction of Method 1 may be represented thus:



3  
Method 2

A mixture of molybdenum hexacarbonyl (5 g.), sublimed sulphur (1.22 g.) and acetylacetone (25 ml., i.e., about 200% excess as a reaction solvent) was gently stirred and boiled under reflux for 6 hours, when the evolution of gas had ceased. The black solid product was collected by filtration, washed with a little benzene and dried in vacuo. The yield was 5.4 g.

The product so recovered had the following analysis: Found: C, 19.04; H, 2.45; Mo, 40.7; S, 22.4%.  $C_5H_7MoO_2S_2$  requires: C, 23.2; H, 2.72; Mo, 28.5; S, 24.7%.

The reaction of Method 2 may be represented thus:



Product M1 was blended into an SAE 90 refined mineral lubricating oil at 1% wt. concentration and the load carrying and anti-wear properties of the composition and of the base oil without M1 were assessed by the well-known 4-ball test, the results being tabulated below.

TABLE 1

| Measurements                | SAE 90 base oil | Base oil plus 1% wt. M1 |
|-----------------------------|-----------------|-------------------------|
| Mean Hertz load (kg.)       | 23              | 31.3                    |
| 2½ seconds delay load (kg.) | 80              | 104                     |
| Welding load (kg.)          | 140             | 200                     |

## EXAMPLE 2

A sample quantity of dithiomolybdenyl stearoylacetone was prepared by the hexacarbonyl/diketone method in accordance with the invention, as described below.

A mixture of molybdenum hexacarbonyl (2.64 g.) and stearoylacetone (20 g.) was heated at 160°–170° C. for 48 hours until evolution of carbon monoxide had slowed appreciably. Sulphur (0.64 g.) was added and the mixture was heated at 150°–160° C. for a further 16 hours. Excess diketone was removed by vacuum distillation, leaving a black solid residue of dithiomolybdenyl stearoylacetone (additive M<sub>2</sub>).

Sufficient of the product was dispersed in benzene and added to a SAE 90 refined mineral oil (as used in Example 1) to give, after removal of benzene by warming under vacuum, a 1 percent by weight blend. The load-carrying and anti-wear properties of the blend were assessed by the 4-ball test, and the results are given in Table 2 below.

## EXAMPLE 3

A sample quantity of dithiomolybdenyl lauroyl-pivaloyl-methanate was prepared by the hexacarbonyl/diketone method in accordance with the invention, as described below.

A mixture of molybdenum hexacarbonyl (2.64 g.) and lauroyl-pivaloyl-methane (17.4 g., 20 ml.) was heated at 160°–170° C. for 48 hours. Sulphur (0.64 g.) was added, and the mixture heated at 150°–160° C. for a further 16 hours. Excess diketone was removed by vacuum distillation leaving a black semi-solid residue of dithiomolybdenyl lauroyl-pivaloyl-methanate (additive M<sub>3</sub>).

Sufficient of the product was dispersed in benzene and added to a SAE 90 refined mineral oil (as used in Example 1) to give, after removal of benzene by warming under vacuum, a 1 percent by weight blend. The load-carry-

ing and anti-wear properties of the blend were assessed by the 4-ball test, and the results are given in Table 2 below.

TABLE 2

| Measurements on 1% wt. blends in SAE 90 oil | Additive M <sub>2</sub><br>$R_1 = \text{Methyl}$<br>$R_2 = \text{n-Heptadecyl}$ | Additive M <sub>3</sub><br>$R_1 = \text{t-Butyl}$<br>$R_2 = \text{n-Undecyl}$ |
|---------------------------------------------|---------------------------------------------------------------------------------|-------------------------------------------------------------------------------|
| Mean Hertz load (kg.)                       | 28.8                                                                            | 30.0                                                                          |
| 2½ second delay load (kg.)                  | 76                                                                              | 100–110                                                                       |
| Welding load (kg.)                          | 200                                                                             | 200                                                                           |
| Initial seizure load (kg.)                  | 70                                                                              | 80                                                                            |

The molybdenum compounds of the present invention when used as additives for lubricating oils are compatible with other, conventional, lubricating oil additives, e.g., antioxidants, V.I. improvers, and detergents.

I claim:

1. A compound of formula



wherein  $R_1$  and  $R_2$  are aliphatic hydrocarbon radicals having 1–20 carbon atoms, and the X's are atoms selected from the group consisting of oxygen and sulphur, at least one of the X's being an oxygen atom.

2. A compound according to claim 1 wherein  $R_1$  and  $R_2$  are alkyl groups.

3. A method of preparing compounds of the formula



wherein  $R_1$  and  $R_2$  are aliphatic hydrocarbon radicals having 1–20 carbon atoms, and the X's are atoms selected from the group consisting of oxygen and sulphur, at least one of the X's being an oxygen atom, which comprises reacting a compound of formula



wherein  $R_1$  and  $R_2$  have the values assigned above, and the X's are atoms selected from the group consisting of oxygen and sulphur, at least one of the X's in each ring being an oxygen atom, with sulphur in an inert atmosphere, and in the presence of a solvent, at an elevated temperature.

4. A method according to claim 3 wherein the reaction is carried out at a temperature within the range 100° C.–200° C.

5. A method of preparing compounds of the formula



wherein  $R_1$  and  $R_2$  are aliphatic hydrocarbon radicals having 1–20 carbon atoms, and the X's are atoms selected from the group consisting of oxygen and sulphur, at

least one of the X's being an oxygen atom, which comprises reacting a compound of formula



wherein the X's, and  $R_1$  and  $R_2$  have the values assigned above, with sulphur and molybdenum hexacarbonyl.

6. A lubricating composition consisting essentially of a blend of a lubricating oil and a compound according to claim 1, the said compound being added in an amount sufficient to improve the lubricating properties of the composition.

7. A lubricating composition according to claim 6 wherein the said compound is added to the extent of 0.1% to 5% by weight of the composition.

References Cited by the Examiner

UNITED STATES PATENTS

2,951,040 8/60 Hugel et al. \_\_\_\_\_ 260—429 X

DANIEL E. WYMAN, Primary Examiner.

UNITED STATES PATENT OFFICE  
CERTIFICATE OF CORRECTION

Patent No. 3,184,410

May 18, 1965

Leslie Bretherick

It is hereby certified that error appears in the above numbered patent requiring correction and that the said Letters Patent should read as corrected below.

Column 1, line 17, for "divide" read -- divided --; column 2, line 13, for "R<sub>1</sub>C(XCH<sub>2</sub>C(X)R<sub>2</sub>)" read -- R<sub>1</sub>C(X)CH<sub>2</sub>C(X)R<sub>2</sub> --; line 53, for "1952" read -- 1962 --.

Signed and sealed this 19th day of October 1965.

(SEAL)

Attest:

ERNEST W. SWIDER  
Attesting Officer

EDWARD J. BRENNER  
Commissioner of Patents